

## UNITED STATES PATENT OFFICE.

WALTER O. SNELLING, OF ALLENTOWN, PENNSYLVANIA. ASSIGNOR TO TROJAN POWDER COMPANY, OF NEW YORK, N. Y., A CORPORATION OF NEW YORK.

## FUSE.

No Drawing.

Application filed March 2, 1925. Serial No. 12,795.

To all whom it may concern:

Be it known that I, WALTER O. SNELLING, a citizen of the United States, residing in Allentown, Lehigh County, Pennsylvania, have invented certain Improvements in Fuses, of which the following is a specification.

My invention relates to improvements in fuse, and the principal object of the invention is to provide an improved fuse for mining and quarrying use.

Fuse of the type commonly employed in mining and quarrying comprises a central core or train of powder surrounded by wrappings of cord or tape and waterproofed by layers of tar, gutta percha or like materials. In use, there is frequently a considerable length of the fuse in contact with the explosive in the bore hole before it reaches the detonating cap, and because of the common tendency of ordinary fuse to burn through the sides or to exude hot tar or other waterproofing material at a temperature in excess of the ignition temperature of the explosive, it frequently happens that the charge of explosive in a bore hole is set on fire by the fuse before the train of powder in the core has transmitted inflammation to the detonator or cap.

The principal object of my present invention is to provide a fuse which will be free from this tendency to ignite powder either by projecting flame or hot gases or by exuding through the sides of the fuse hot tar, or other waterproofing materials.

I have discovered that by employing, instead of the usual waterproofing materials, a mixture comprising an unvulcanized but vulcanizable material, I am able to materially modify or entirely eliminate the aforescribed "side-spitting" tendency of fuse with its attendant objectionableness. By vulcanizable material I mean one which upon being heated will develop a change in its physical characteristics tending towards solidification, or will become less fluid rather than more fluid. By vulcanization is meant the process of becoming less fluid or more solid with increasing temperature in contradistinction to the increased fluidity with heating of the usual plastic waterproofing materials.

In the practice of my invention, I may employ many materials as the waterproofing

agent, although I prefer to employ mixtures comprising rubber and sulfur, or gutta percha and sulfur either with or without an accelerator of vulcanization. In general, I may employ any material which has waterproofing properties and which is plastic and flexible when not heated, but which becomes solid and non-fluid when heated to predetermined temperatures.

As an example of a waterproofing agent made in accordance with my invention, I may employ a coating consisting of a mixture of asphalt, tar or like material with unvulcanized rubber and sulfur, preferably in association with an accelerator of vulcanization for the purpose of causing the vulcanizing reaction to go on at a lower temperature. The amount of rubber present in the tar-asphalt composition may be comparatively small, for example from 5% to 20%, and there should be sufficient sulfur to vulcanize this rubber and to leave a considerable excess for the tar-asphalt composition. As examples of accelerators of vulcanization that may be successfully employed, I may use hexamethylenetetramine, quinoline, piperidine, &c., and the accelerator may be present in amount up say to 1% of the composition, the amount being determined by the rapidity with which it is desired that the vulcanization take place. It should be understood, however, that the accelerator may be entirely omitted and I wish to place no limitation on the amounts employed.

In applying this composition to the fuse, the latter may be passed through the composition in the same manner as when the usual tar-asphalt composition is employed, care being taken, however, to melt the mixture at a temperature below that required for vulcanization.

Although in the above example I have described a vulcanizable material requiring for vulcanization the presence of a vulcanizing agent, it will be understood that I do not limit myself to this particular class of vulcanizable material. I may employ for example such materials as tung oil, commonly known as China wood oil, which hardens when heated, and this material can replace a mixture of rubber and sulfur in the waterproofing compound. It is also well known that phenol formaldehyde condensation products, such as bakelite varnish,

harden on the application of heat, and resins of this type have been used with success as waterproofing agents in connection with the present invention.

5. A fuse made in accordance with this invention will preferably comprise the usual central powder core or train and a surrounding protective cover having the normal water-proofing characteristics of fuse as 65  
10 manufactured before my invention. When the powder core burns, however, the intense heat thus produced exceeds the vulcanization temperature of the rubber sulfur mixture or other vulcanizable agent in the waterproof- 70  
15 ing composition, and the vulcanization of this material forms a solid body that holds together the other constituents of the composition and prevents the throwing off or exuding of these constituents from the fuse. 75  
20 I have found that it is of material assistance in the application of my invention to employ wrappings of paper around my waterproofing composition and inside the final counteracting of my fuse. I preferably 80  
25 employ one wrapping of paper in the form of a tube of paper, the two edges of the paper being slightly overlapped, and a second wrapping of paper in the form of a spiral wrapping. I may place my waterproof- 85  
30 ing agent within the innermost of the two paper wrappings, or I may place my waterproofing agent between the two wrappings.

I claim:

- 35 1. Fuse comprising a powder core, and a waterproofing cover for said core including a substance tending to vulcanize with increasing temperature.
2. Fuse comprising a powder core, and a 40 waterproofing cover for said core including an unvulcanized vulcanizable material.
3. Fuse comprising a powder core, and a bitumen waterproofing cover comprising an unvulcanized vulcanizable material.
- 45 4. Fuse comprising a powder core, and a waterproofing cover for said core including an unvulcanized vulcanizable material and a vulcanizing agent.
5. Fuse comprising a powder core, and a 50 protective cover for said core comprising unvulcanized rubber and a vulcanizing agent.
6. Fuse comprising a powder core, and a protective cover for the core comprising an 55 unvulcanized vulcanizable material, a vulcanizing agent, and a vulcanization accelerator.
7. Fuse comprising a powder core, and a protective cover for said core including 60 China wood oil.
8. Fuse comprising a powder core, and a protective cover for said core including an unhardened synthetic resin.
9. A waterproof coating material for fuse

comprising an unvulcanized vulcanizable material.

10. A coating material for fuse comprising a plastic waterproofing substance in admixture with an unvulcanized vulcanizable material.

11. A coating material for fuse comprising a plastic bitumen substance containing an unvulcanized vulcanizable material.

12. A coating material for fuse comprising a plastic waterproofing substance, unvulcanized rubber and sulfur.

13. A coating material for fuse comprising a plastic waterproofing substance, unvulcanized rubber, and sulfur in excess of the amount required to vulcanize the said rubber.

14. A coating material for fuse comprising a plastic waterproofing substance containing 5% to 20% of unvulcanized rubber, and sulfur in excess of the amount required to vulcanize said rubber.

15. A coating material for fuse comprising unvulcanized rubber and sulfur.

16. A coating material for fuse comprising unvulcanized rubber and sulfur in excess of the amount required to vulcanize said rubber.

17. A coating material for fuse comprising an unvulcanized vulcanizable material and a vulcanizing agent.

18. A coating material for fuse comprising a vulcanizable material and a vulcanization accelerator.

19. A coating material for fuse comprising unvulcanized rubber, sulfur and hexamethylenetetramine.

20. A coating material for fuse comprising an unvulcanized vulcanizable material, a vulcanizing agent, and a vulcanization accelerator.

21. A coating material for fuse comprising China wood oil.

22. A coating material for fuse comprising an unhardened synthetic resin.

23. The method of manufacturing fuse, which consists in taking a powder core and covering said core with a waterproofing material including an unvulcanized vulcanizable material.

24. The method of preventing sidesplitting in fuse comprising a waterproof cover, which consists in incorporating in said cover an unvulcanized vulcanizable material.

25. The method of manufacturing fuse which consists in preparing a waterproofing material containing an unvulcanized vulcanizable material, heating the material to a liquid or plastic condition at a temperature below that required for vulcanization, and applying the material to a powder core in the form of a protective cover.

WALTER O. SNELLING,